

Dec. 1, 1925.

1,563,980

G. W. HEISE

GALVANIC CELL OF THE COPPER OXIDE TYPE

Filed May 27, 1924



Inventor:

George W. Heise,

By *Byers, Townsend & Bruckenstein*,  
Attorneys.

## UNITED STATES PATENT OFFICE.

GEORGE W. HEISE, OF BAYSIDE, NEW YORK, ASSIGNOR TO NATIONAL CARBON COMPANY, INC., A CORPORATION OF NEW YORK.

## GALVANIC CELL OF THE COPPER-OXIDE TYPE.

Application filed May 27, 1924. Serial No. 716,267.

To all whom it may concern:

Be it known that I, GEORGE W. HEISE, a citizen of the United States, residing at Bayside, in the county of Queens and State 5 of New York, have invented certain new and useful Improvements in Galvanic Cells of the Copper-Oxide Type, of which the following is a specification.

This invention relates to improvements in 10 cells of the soluble metal-caustic alkali-depolarizing oxide type, especially copper oxide cells. A primary purpose of the invention is to prevent the adverse effect of dissolved copper. This is preferably accomplished by fixing the dissolved copper in 15 the form of compounds having no substantial detrimental action in the cell.

To this end I have devised improved 20 coatings, wrappings, or the like, which are interposed between the copper oxide and the caustic electrolyte. These may have the dual function of fixing dissolved copper and 25 of preventing the escape of copper oxide particles. Alternatively, suitable materials may be added to the electrolyte to react with 30 copper in solution. The invention includes other novel and advantageous features, which will appear from the following description.

It has heretofore been proposed to secure 35 a paper wrapping or lining by means of an adhesive to copper oxide containers. Frequently the action of the caustic electrolyte loosens the paper and causes it to break 40 away from the container. In the prior processes referred to, this has not been considered an objection, because the only function sought from the paper was that of retaining the oxide during the period before the filled container was put into service.

I have discovered that a layer of cellulosic 45 material of special type, or its equivalent, has an additional function of great importance which is operative throughout the 50 service life of the cell. This function, as noted above, is the retention of dissolved copper. My experiments have demonstrated that copper oxide is dissolved from the depolarizer by the electrolyte and that 55 the copper in solution is decidedly detri-

mental. Copper appears to be deposited upon the zinc, causing wasteful local action.

I have discovered, further, that the dissolved copper reacts with certain materials to form compounds harmless to the cell. 55 Among these materials are cellulosic compounds, for example wood pulp and starch, and nitrogenous bodies of the type of gluten. In the case of wood pulp it seems probable that cellulose hydrates are formed, and that 60 these hydrates combine with the dissolved copper compounds to form a gel insoluble in the alkali electrolyte. The invention is of course in no way dependent upon the theory of reaction. 65

With reference to the use of starch, I am aware that this material has been employed as a gelatinizing agent for caustic electrolyte. For the purposes of the present invention, the quantity of starch required is 70 far lower than that heretofore used.

In view of the facts stated, it is highly desirable to provide a permanent coating or lining which can be depended upon to prevent dissolved copper from passing beyond 75 the confines of the depolarizing body. I have attained this object, in one embodiment of the invention, by forming a paper coating directly upon the copper oxide element or the container in which the copper 80 oxide is to be placed.

It is preferred to form the paper coating in the following manner: Cellulosic material, preferably wood pulp such as is ordinarily used in paper making, is beaten up 85 with sufficient caustic alkali solution to form a gelatinous or pasty mass. This may be applied to the containers or coherent bodies of copper oxide and on drying will form a permanently adherent coating. When containers are used the depolarizer may be placed therein as usual. If the depolarizer is to be tamped in under considerable pressure, it is desirable to provide a removable 90 supporting sleeve adjacent to the container 95 wall to prevent rupture of the coating or lining.

The strength of the caustic solution used to gelatinize the wood pulp suspension may be varied widely. A 2% aqueous solution 100

of sodium hydroxide may be used with advantage. Less than 0.7% alkali does not ordinarily give good results. Solutions stronger than 2% are advantageous in causticizing the pulp, but ordinarily give a product which is difficult to use. The retained caustic in such case frequently makes the pulp hygroscopic and corrosive when applied to metal containers. These difficulties may be avoided, however, by neutralizing the greater portion of the alkali prior to the papering operation. Other gelatinizing agents, for example zinc chlorid, may be used instead of an alkali metal hydroxide. 10 The causticized product may be applied in various ways either to sheet metal, finished containers, or coherent depolarizing bodies. It may be spread or brushed on, or may be sprayed. The appearance of the 20 containers may be improved by floating a thin suspension of the pulp over a rough first coat of thick pulp.

While causticized wood pulp is generally preferred, other forms of cellulosic material 25 or its equivalent may be used. For example, the depolarizing bodies may be coated with an adhesive and rolled in wood fiber to form a surface layer.

For illustrative applications of the present invention, reference is to be made to the accompanying drawing, in which:

Fig. 1 is a vertical section through a cell 30 provided with a perforated depolarizer container having a paper coating;

Fig. 2 is a perspective view of a metal blank with a similar coating; and

Fig. 3 is a perspective view of a paper-coated, agglomerated mass of copper oxide, the coating being partly broken away.

In the drawing, reference numeral 1 denotes a perforated container suspended by rod 2 from cover 3 and immersed in caustic alkali electrolyte 4. The illustration shows a copper oxide cell of a commercial type.

The invention may of course be applied to other kinds of cells.

The container 1 is covered with a layer of cellulosic material 5, or equivalent substance. This is preferably applied as an exterior coating, as shown, and by the process previously described. It may, however, be applied as a lining, or may merely fill the perforations.

While the cellulosic material may be applied to finished containers, there is considerable advantage in coating perforated sheet metal prior to shaping it. As shown in Fig. 2, a layer 6 of causticized wood pulp may be applied to a perforated metallic sheet 7 adapted for use in making up containers. The layer 6 does not interfere with the shaping of the metal nor become detached during that process.

As shown in Fig. 3, cellulosic material 8 may be applied to an agglomerated mass of

copper oxide 9. Various other applications of the material may be made.

Unlike paper secured to the container by an adhesive, the paper formed in situ as described does not become detached even after 70 long immersion in electrolyte. It has, moreover, a much greater power of fixing dissolved copper than has the paper heretofore used. This is probably due to the fact that it is applied in causticized state. 75

I prefer to use the new form of paper coating in all cases, but it is within the scope of the invention to apply a cellulosic coating of any suitable kind to coherent bodies of copper oxide. So far as I am aware, 80 cellulosic material has heretofore been used in copper oxide cells only in connection with containers for the purpose of obstructing perforations, or for gelatinizing the electrolyte, as referred to above. The present invention attains the novel result of preventing copper from passing into liquid electrolyte from coherent depolarizing bodies. The invention includes further the improved cellulosic coating described, as applied either 85 to coherent depolarizers, containers, or in other suitable ways. 90

I do not claim herein the coating or lining of copper oxide containers with paper in preformed sheets, the filling of the perforations in such containers with cellulosic material, or broadly the use of proteins, gums, and resins in the electrolyte. Such subject matter is described and claimed respectively in applications Serial Nos. 610,844, filed 95 January 5, 1923, 606,520, filed December 12, 1922, and 619,464, filed February 16, 1923, in each of which I am a co-inventer. 100

I claim:

1. In a galvanic cell with copper oxide 105 depolarizer and fluid caustic electrolyte, a material adapted to chemically fix dissolved copper and operatively disposed with respect to the depolarizer.

2. In a galvanic cell with copper oxide 110 depolarizer and caustic electrolyte, a coating upon the depolarizer and adapted to chemically fix dissolved copper.

3. A coherent copper oxide depolarizer having thereon a coating of material adapted 115 to chemically fix dissolved copper.

4. A copper oxide depolarizing body having thereon a coating of causticized cellulosic material.

5. A copper oxide depolarizing body having thereon a coating of causticized wood pulp. 120

6. A copper oxide container comprising perforated sheet metal having thereon a coating of causticized cellulosic material. 125

7. Process of preventing the detrimental effect of dissolved copper in fluid caustic electrolyte, comprising utilizing in the cell a material adapted to chemically fix such copper in harmless form. 130

8. Process of coating copper oxide depolarizing bodies, comprising applying thereto a layer of causticized cellulosic material.
9. Process of forming an adherent paper coating on copper oxide depolarizing bodies, comprising applying thereto gelatinous causticized wood pulp.
10. Process of forming a surface layer on perforated sheet metal adapted to be shaped into copper oxide containers, comprising applying thereto causticized wood pulp.

11. Process of coating copper oxide containers, comprising distributing thereon causticized cellulosic material adapted to form a paper-like layer.

In testimony whereof, I affix my signature.  
GEORGE W. HEISE.